

## UNITED STATES PATENT OFFICE

2,206,847

## ALLOY STEEL

Clarence H. Lorig, Columbus, Ohio, assignor to  
Battelle Memorial Institute, Columbus, Ohio, a  
corporation of Ohio

No Drawing. Original application July 11, 1938,  
Serial No. 218,633. Divided and this applica-  
tion March 13, 1940, Serial No. 323,791

4 Claims. (Cl. 75—126)

My invention relates to an alloy steel. It re-  
lates more particularly to a steel which has a  
high sensitivity to work-hardening.

One of the objects of this invention is the  
provision of an alloy steel which may be used  
for producing wrought and cast articles having  
a high capacity for work-hardening.

A further object of this invention is the pro-  
vision of an alloy steel used for producing articles  
10 having a high sensitivity to work-hardening that  
possesses great strength and toughness.

Still another object of this invention is the pro-  
vision of a work-hardenable alloy steel product  
15 having great strength and toughness.

Other objects and advantages of my invention  
will become apparent from the following descrip-  
tion and claims.

This application is a division of my co-pending  
application Serial No. 218,633, filed July 11, 1938.

20 I have found that the manganese content of  
the 11 to 14 per cent manganese work-harden-  
ing steel can be substantially reduced by alloying  
with copper and molybdenum and that the sta-  
bilization of the austenite structure of this type  
25 of work-hardening steel can be accomplished by  
employing much lower manganese contents when  
both copper and molybdenum are present. The  
composition range in which the specified advan-  
tages were found is as follows:

30 Carbon 0.50 to 1.7 per cent, manganese 2.0 to  
9.0 per cent, copper 1 to 5 per cent, molybdenum  
traces to 3.0 per cent, the remainder being iron

1.5 per cent silicon may be present in the steel.  
Some chromium may be used to further increase  
the wear resistance and to raise the yield and  
tensile strengths of the steel. For this purpose,  
however, less than 3 per cent of chromium is  
satisfactory.

I have discovered the combining of manganese,  
copper, molybdenum, and carbon in the propor-  
tions indicated makes steel very sluggish to allo-  
tropic changes, so that in the water-quenched 10  
condition or after cooling quickly in air it stays  
in the austenitic state. However, the changes  
are not too sluggish, so that cold-working will  
cause the worked surface of the steel to transform  
from soft austenite to extremely hard martensite. 15  
High sensitivity to work-hardening is obtained  
when the transformation of austenite to marten-  
site by cold working is rapid. In applications  
where my steel is subjected to combined pound-  
ing or impact and abrasion, the transformation is 20  
rapid and the steel resists wear to a remarkable  
degree. New, hard surfaces form as rapidly as  
the earlier martensitic surfaces are removed by  
wear.

The following table lists the hardness of a 25  
number of steels after different heat treatments  
and shows the relative work-hardenability of the  
steels by the difference in Rockwell "C" hardness  
of the unworked surface and the hardness at the  
bottom of a Brinell impression where the metal 30  
is worked.

| Steel No. | C, percent | Mn, percent | Cu, percent | Mo, percent | Hardness after various heat treatments |              |                              |                  |                          |                              |                  |              |                              |
|-----------|------------|-------------|-------------|-------------|----------------------------------------|--------------|------------------------------|------------------|--------------------------|------------------------------|------------------|--------------|------------------------------|
|           |            |             |             |             | 1,650° F. water quenched               |              | 1,650° F. air cooled         |                  | 1,650° F. furnace cooled |                              |                  |              |                              |
|           |            |             |             |             | Brinell hardness                       | Rockwell "C" |                              | Brinell hardness | Rockwell "C"             |                              | Brinell hardness | Rockwell "C" |                              |
|           |            |             |             |             |                                        | Surface      | Bottom of Brinell impression |                  | Surface                  | Bottom of Brinell impression |                  | Surface      | Bottom of Brinell impression |
| 1         | 0.5        | 1.5         | 3.0         | 0.5         | 578                                    | 61           | 67                           | 549              | 55                       | 60                           | 361              | 39           | 44                           |
| 2         | 1.2        | 3.0         | 3.0         | .5          | 200                                    | 24           | 43                           | 210              | 24                       | 43                           | 477              | 49           | 54                           |
| 3         | 1.2        | 3.0         | 3.0         | 3.0         | 232                                    | 32           | 46                           | 241              | 29                       | 44                           | 531              | 38           | 49                           |
| 4         | 1.2        | 2.0         | 5.0         | 1.0         | 245                                    | 35           | 56                           | 285              | 39                       | 52                           | 477              | 41           | 50                           |
| 5         | 1.25       | 2.0         | 3.0         | 0.5         | 255                                    | 33           | 50                           | 401              | 42                       | 52                           | 409              | 39           | 47                           |
| 6         | 1.25       | 4.0         | 4.0         | .5          | 224                                    | 10           | 34                           | 242              | 20                       | 39                           | 518              | 49           | 54                           |
| 7         | 1.25       | 5.0         | 3.0         | .5          | 217                                    | 14           | 28                           | 228              | 15                       | 36                           | 454              | 38           | 49                           |
| 8         | 1.25       | 5.0         | 3.0         | .75         | 229                                    | 23           | 36                           | 232              | 18                       | 41                           | 429              | 43           | 50                           |
| 9         | 1.25       | 6.0         | 3.0         | Trace       | 221                                    | 22           | 38                           | 225              | 20                       | 42                           | 404              | 41           | 47                           |
| 10        | 1.25       | 7.0         | 3.0         | Trace       | 228                                    | 24           | 40                           | 246              | 24                       | 46                           | 385              | 38           | 46                           |
| 11        | 1.26       | 7.0         | 3.0         | .50         | 229                                    | 23           | 39                           | 229              | 18                       | 40                           | 378              | 40           | 54                           |
| 12        | 1.25       | 7.0         | 1.5         | .50         | 224                                    | 18           | 38                           | 241              | 18                       | 42                           | 398              | 39           | 55                           |
| 13        | 1.25       | 4.0         | 1.0         | .50         | 226                                    | 20           | 35                           | 256              | 21                       | 43                           | 518              | 40           | 54                           |
| 14        | 1.25       | 4.0         | 2.0         | 1.00        | 229                                    | 20           | 34                           | 232              | 16                       | 40                           | 560              | 52           | 58                           |
| 15        | 1.50       | 3.0         | 3.0         | .5          | 269                                    | 28           | 43                           | 354              | 33                       | 46                           | 499              | 49           | 54                           |
| 16        | 1.00       | 3.0         | 3.0         | .5          | 215                                    | 27           | 42                           | 205              | 20                       | 44                           | 518              | 50           | 54                           |
| 17        | 0.75       | 3.0         | 3.0         | .5          | 477                                    | 54           | 60                           | 435              | 50                       | 56                           | 514              | 52           | 54                           |
| 18        | 1.25       | 5.0         | 3.0         | .25         | 224                                    | 18           | 39                           | 234              | 16                       | 41                           | 441              | 42           | 51                           |

together with the usual amounts of silicon, sul-  
fur, and phosphorus normally in steel. From  
traces up to 0.15 per cent phosphorus, from traces  
up to 0.10 per cent sulfur, and from traces up to

As compared with the above steels, a 14 per  
cent manganese, 1.25 per cent carbon steel after  
quenching in water from 1900° F. had a Brinell  
hardness of 175, a Rockwell "C" hardness of 13 60

on the unworked surface, and a Rockwell "C" hardness of 40 on the bottom of a Brinell impression.

Water-quenched specimens of steel coming within the range of composition which I previously specified will have a Brinell hardness in excess of 210. In the range of composition centering around 1.00 to 1.5 per cent carbon, 3 to 7 per cent manganese, 1 to 4 per cent copper, and from traces to 1.00 per cent molybdenum, which is my preferred range, Brinell hardnesses of water-quenched specimens are from 210 to about 260, or values that are substantially above the value for the 14 per cent manganese steel. The higher hardness is also associated with higher tensile strength. In this range of preferred composition, the steel transforms very rapidly at the surface from soft austenite to extremely hard martensite on cold working, as shown by the difference in Rockwell "C" hardness of the un-worked surface and of the bottom of the Brinell impression of water-quenched material. The air-cooled steel in the same range of composition is also austenitic and also transforms to martensite on cold-working. After furnace cooling, the steel is partially or fully martensitic and hard.

Below the preferred range of carbon and alloy contents, it is more difficult to obtain the steel in the austenitic state and thus make it work-hardenable without an extremely drastic quenching from high temperatures.

Carbon has a very powerful influence on stabilizing austenite and in making the steel suitable for work-hardening. With carbon contents below 1.0 per cent, it becomes increasingly difficult to develop work-hardening properties in the steel. A suitable carbon range is quite narrow, as I have found that with carbon contents above 1.50 per cent the steel not only becomes harder in the quenched state but becomes less satisfactory for work-hardening. Carbon is, therefore, an important element which must be kept within close limits in my steel.

Copper and molybdenum augment carbon and manganese in retaining austenite. Both copper and molybdenum retard the rate of transformation of gamma iron to alpha iron, and particularly so in the presence of manganese and carbon. Consequently, I have found it possible to reduce the manganese in austenitic work-harden-  
ing steel as much as 75 per cent by alloying with copper and molybdenum. 1 to 5 per cent copper and from traces to 3 per cent molybdenum make possible a reduction in the amount of manganese of from 1 to 3 times the total percentage of copper and molybdenum added. Too high a molybdenum content like too high a carbon content tends to harden the steel when water-quenched, making it less susceptible to work-hardening. For that reason, I prefer to limit its use below 3 per cent. Excellent results are obtained with 0.25 per cent to 0.50 per cent molybdenum.

In addition to its influence on stabilizing austenite, copper increases the strength of the steel. In the range of composition in which the steel is machinable, copper also aids the machinability.

An important advantage of my alloy steel over the high-manganese steel is that in the range of composition of about 2 to 4 per cent of copper, 5 to 7 per cent of manganese, traces to 0.50 per cent of molybdenum, and 1.00 to 1.50 per cent of carbon the steel is machinable with ordinary carbon and high-speed steel tools. The machin-

ability of the steel in this range of composition constitutes quite an advance in the art, as the high-manganese steel can be machined only with the greatest difficulty by special carbide tools or by grinding. To effect machinability, the steel is cooled slowly as, for example, in a well-insulated furnace. The following table shows the maximum permissible machining speed for a number of compositions after they were cooled slowly in a furnace from 1650° F. Cuts were made on a lathe using a high-speed tool at a feed of  $\frac{1}{16}$ -inch per revolution. A specimen  $\frac{3}{8}$ -inch square was reduced to  $\frac{3}{4}$ -inch round in one cut.

| C, percent | Mn, percent | Mo, percent | Cu, percent | Brinell, hardness | Maximum permissible machining speed, R. P. M. |
|------------|-------------|-------------|-------------|-------------------|-----------------------------------------------|
| 1.25       | 3.0         | Trace       | 3.0         | 321               | 167                                           |
| 1.25       | 6.0         | Trace       | 3.0         | 406               | 100                                           |
| 1.25       | 7.0         | Trace       | 3.0         | 380               | 120                                           |
| 1.25       | 5.0         | Trace       | 3.0         | 415               | 87                                            |
| 1.25       | 2.0         | 0.5         | 3.0         | 415               | 45                                            |

After machining, the steel can be made work-hardenable by heat-treating and liquid or air-quenching.

The higher quenching temperatures up to a certain maximum were found to improve the ductility of the steel considerably. A quenching temperature above 1800° F. was found to be most satisfactory, although it is possible to quench from lower temperatures.

Mechanical properties of the steel in the preferred range of composition are excellent. Its toughness was demonstrated with key-hole notched Charpy specimens water-quenched and tested for impact in a machine of 120 ft.-lb. capacity. The specimens absorbed the full 120 ft.-lb. of energy of the machine with a single blow without breaking. Any steel coming within the range of composition specified hereinbefore will have an impact strength in excess of 30 ft.-lbs.

The alloy steel is suitable for services requiring high resistance to the combination of repeated blows or impact and abrasion. Articles such as plates for jaw crushers, ball mill liners, roll shells, dipper teeth, caterpillar shoes, etc., can be made from my alloy.

Having thus described my invention, what I claim is:

1. An alloy steel consisting of 0.50 to 1.7 per cent carbon, 2.0 to 9.0 per cent manganese, 1 to 5 per cent copper, traces to 3 per cent molybdenum, traces to 0.15 per cent phosphorus, traces to 0.10 per cent sulfur, traces to 1.5 per cent silicon, up to 3.0 per cent chromium, and the remainder substantially all iron, said alloy steel being austenitic after quenching from a high temperature.

2. An alloy steel containing 0.50 to 1.7 per cent carbon, 2.0 to 9 per cent manganese, 1 to 5 per cent copper, traces to 3 per cent molybdenum, traces to 0.15 per cent phosphorus, traces to 0.10 per cent sulfur, traces to 1.5 per cent silicon, up to 3.0 per cent chromium, the remainder being substantially iron, said steel being austenitic and work-hardenable after quenching from a high temperature and having a Brinell hardness in excess of 210 and an impact strength in excess of 30 ft.-lbs.

3. An alloy steel containing 1.00 to 1.5 per cent carbon, 3 to 7 per cent manganese, 1 to 4 per cent copper, traces to 1.00 per cent molyb-

5 denum, traces to 0.15 per cent phosphorus, traces to 0.10 per cent sulfur, traces to 1.5 per cent silicon, up to 3.0 per cent chromium, and the balance substantially iron, said steel being austenitic and work-hardenable after quenching from a high temperature and having a Brinell hardness ranging from 210 to 260 and having an impact strength in excess of 120 ft.-lbs.

4. An alloy steel consisting of 1.00 to 1.5 per cent carbon, 3 to 7 per cent manganese, 1 to 4 per cent copper, traces to 1.00 per cent molybdenum, traces to 0.15 per cent phosphorus, traces to 0.10 per cent sulfur, traces to 1.5 per cent silicon, up to 3.0 per cent chromium, and the remainder substantially all iron.

CLARENCE H. LORIG.